



US005538577A

# United States Patent [19]

Negoro

[11] Patent Number: 5,538,577

[45] Date of Patent: Jul. 23, 1996

[54] **THERMAL TRANSFER RECORDING MATERIAL**

[75] Inventor: **Toshihiko Negoro**, Osaka, Japan

[73] Assignee: **Fujicopian Co., Ltd.**, Osaka, Japan

[21] Appl. No.: **346,095**

[22] Filed: **Nov. 29, 1994**

[30] **Foreign Application Priority Data**

Nov. 30, 1993 [JP] Japan ..... 5-300282

[51] Int. Cl.<sup>6</sup> ..... B41M 5/26; B41M 5/40

[52] U.S. Cl. ..... 156/235; 428/195; 428/341;  
428/913; 428/914

[58] Field of Search ..... 8/471; 428/195,  
428/913, 914, 341; 503/227; 156/235

[56] **References Cited**

FOREIGN PATENT DOCUMENTS

63-317386 12/1988 Japan ..... B41M 5/26

Primary Examiner—B. Hamilton Hess  
Attorney, Agent, or Firm—Fish & Neave

[57] **ABSTRACT**

A thermal transfer recording material comprising a foundation, and (A) a coated area of at least one heat-meltable ink and (B) a coated area of a release agent or a release composition containing a release agent provided on the foundation, the coated area (A) and the coated area (B) being repeatedly arranged in a side-by-side relation on one side of the foundation, the release agent being at least one member selected from the group consisting of a silicone oil, an alkyl phosphate, a fluorine-containing surface active agent, a silicone resin, a silicone-modified urethane resin, a silicone-modified acrylic resin and a fluorine-containing resin. The thermal transfer recording material is favorably used in a reheating method wherein the heat-meltable ink is transferred onto a receptor, especially a receptor having a porous surface layer, and the ink image formed on the receptor is heated under the condition that the release agent-coated area (B) of the recording material is superimposed on the ink image.

7 Claims, 1 Drawing Sheet



FIG. 1



FIG. 2



## THERMAL TRANSFER RECORDING MATERIAL

### BACKGROUND OF THE INVENTION

The present invention relates to a thermal transfer recording material. More particularly, it relates to a thermal transfer recording material useful for forming ink images having a smooth surface on a receptor having a porous surface layer.

Heretofore there was proposed a thermal transfer recording method using a thermal transfer recording material wherein a coated area of a heat-meltable ink and an uncoated area thereof are repeatedly arranged in a side-by-side relation on one side of a foundation. The method comprises: selectively transferring the heat-meltable ink of the coated area by means of a thermal head to form ink images on a receptor paper, superimposing the uncoated area of the ink on the recording material onto the image-bearing surface of the receptor paper, and heating the ink images by means of the thermal head to permit the ink of the images to penetrate voids between the fibers of the receptor paper, thereby giving ink images having excellent abrasion resistance and durability (Japanese Unexamined Patent Publication No. 103488/1989). Hereinafter this method is referred to as reheating method.

On the other hand, there was developed as a receptor for use with a thermal transfer recording material a receptor having a porous surface layer (hereinafter referred to as porous surface receptor) wherein a resinous layer having a large number of minute pores is formed on a film substrate (Japanese Unexamined Patent Publication No. 41287/1990).

Although the porous surface receptor has been subjected to a smoothing treatment in the production thereof, the surface of the receptor is still uneven and poor in smoothness. Accordingly, the ink image formed on the receptor has a uneven surface, which causes a diffused reflection, resulting in a low image density, or a poor color reproduction with respect to full-color image.

In order to settle the above problems, the present inventor has attempted to smooth the surface of the ink image formed on the porous surface receptor by applying the above-mentioned reheating method. However, in the reheating step, a phenomenon occurred that some portion of the ink of the images adheres to the uncoated area of the recording material transfer to the recording material. Hereinafter, the phenomenon is referred to as reverse transfer. The reverse transfer degrades the quality of the ink image.

It is an object of the present invention to provide a thermal transfer recording material for use in the aforesaid reheating method which does not cause the reverse transfer in the reheating step.

This and other objects of the present invention will become apparent from the description hereinafter.

### SUMMARY OF THE INVENTION

The present invention provides a thermal transfer recording material comprising a foundation, and (A) a coated area of at least one heat-meltable ink and (B) a coated area of a release agent or a release composition containing a release agent provided on the foundation, the coated area (A) and the coated area (B) being repeatedly arranged in a side-by-side relation on one side of the foundation, the release agent being at least one member selected from the group consisting of a silicone oil, an alkyl phosphate, a fluorine-containing surface active agent, a silicone resin, a silicone-modified

urethane resin, a silicone-modified acrylic resin and a fluorine-containing resin.

### BRIEF DESCRIPTION OF THE DRAWINGS

FIG. 1 is a partial plan view showing an example of the thermal transfer recording material of the present invention.

FIG. 2 is a partial plan view showing another example of the thermal transfer recording material of the present invention.

### DETAILED DESCRIPTION

The thermal transfer recording material of the present invention is preferably used in the following way:

In a thermal transfer printer, the coated area of the heat-meltable ink on the thermal transfer recording material is superimposed onto a receptor and the heat-meltable ink is selectively melt-transferred onto the receptor by heating from the back side of the recording material with a heating means such as a thermal head, giving an ink image on the receptor. Then the release agent-coated area of the same recording material is superimposed onto the image-receiving surface of the receptor on which the ink image has been formed and the ink image is heated from the back side of the recording material with the heating means such as a thermal head. In this reheating treatment step, the ink image is heated while contacting the release agent-coated area and, hence, the ink of the image is not transferred to the recording material, namely the reverse transfer does not occur. The ink of the image is again softened or melted by the reheating treatment, with which the depressed portions of the surface of the receptor is filled, resulting in smoothed surface of the ink image. The thus smoothed surface of the ink image causes much less diffused reflection, resulting in an increased image density. In the case that the ink image is a multi-color or full-color image, the reheating treatment improves the color reproduction of the image.

The thermal transfer recording material of the present invention will be explained by referring to the drawings.

FIG. 1 is a partial plan view showing an example of the thermal transfer recording material of the present invention.

The thermal transfer recording material illustrated in FIG. 1 is used for forming a monochromatic image. A coated area 2 of a heat-meltable ink and a coated area 3 of a release agent or a release composition are alternately repeatedly arranged in a side-by-side relation on a foundation 1 in the longitudinal direction thereof.

Usable as the ink for the coated area 2 are a black ink as well as inks in various colors such as blue, red, green and yellow.

Usually the size of the ink-coated area 2 is substantially the same as the size of the release agent-coated area 3. For example, in the case of a thermal transfer recording material having a small width for use with a serial type thermal transfer printer, usually the coated area 2 and the coated area 3 each have a size corresponding to one printing line (or a size corresponding to plural printing lines for a printer capable of simultaneously printing plural lines). In the case of a thermal transfer recording material having a large width for use with a line type thermal transfer printer, usually the coated area 2 and the coated area 3 each have a size corresponding to a receptor.

The thermal transfer recording material illustrated in FIG. 2 is used for forming a multi-color or full-color image composed of plural colors. On a foundation 11 are alter-

nately repeatedly arranged a set of a plurality of different color coated areas, for example, a coated area 12Y of a yellow ink, a coated area 12M of a magenta ink and a coated area 12C of a cyan ink, and a coated area 13 of a release agent or a release composition in a side-by-side relation in the longitudinal direction of the foundation 11.

With use of the recording material, at least two of the yellow ink, magenta ink and cyan ink are superimposingly transferred to a receptor in a predetermined order to give a color image on the basis of subtractive color mixture. Accordingly, in usual cases, one coated area 13 is provided relative to one set of the coated areas 12Y, 12M and 12C. Usually the size of each of the coated areas 12Y, 12M and 12C is substantially the same as the size of the release agent-coated area 13. For example, in the case of a thermal transfer recording material having a small width for use with a serial type thermal transfer recording material, usually the coated areas 12Y, 12M and 12C and the coated area 13 each have a size corresponding to one printing line (or a size corresponding to plural printing lines for a printer capable of simultaneously printing plural lines). In the case of a thermal transfer recording material having a large width for use with a line type thermal transfer printer, usually the coated areas 12Y, 12M and 12C and the coated area 13 each have a size corresponding to a receptor.

In the aforesaid thermal transfer recording material for color image formation, a repeating unit U is composed of one set of the coated areas 12Y, 12M and 12C of respective color inks and one coated area 13. The order of arrangement of the coated areas 12Y, 12M and 12C of respective color inks in the repeating unit U may be determined depending upon the order of transfer of the respective color inks. The release agent-coated area 13 is usually arranged so that it appears lastly in the repeating unit U relative to the traveling direction of the recording material. The repeating unit U may further include a coated area of a black ink.

As the foundation for the recording material of the present invention, usable are polyester films such as polyethylene terephthalate film, polyethylene naphthalate film and polyarylate film, polycarbonate films, polyamide films, aramid films and other various plastic films commonly used for the foundation of ink ribbons of this type. Thin paper sheets of high density such as condenser paper can be used. The thickness of the foundation is preferably within the range of about 1 to 10  $\mu\text{m}$ , more preferably about 1 to 7  $\mu\text{m}$ , for better heat conduction.

On the back side (the side adapted to come into slide contact with a thermal head) of the foundation may be formed a conventionally known stick-preventive layer. Examples of the material for the stick-preventive layer include various heat-resistant resins such as silicone resin, fluorine-containing resin and nitrocellulose resin, and other resins modified with these heat-resistant resins such as silicone-modified urethane resins and silicone-modified acrylic resins, and mixtures of the foregoing heat-resistant resins and lubricating agents.

As the heat-meltible ink used in the present invention, there can be employed any of conventional ones comprising a coloring agent and a heat-meltible vehicle without no particular limitation. The heat-meltible vehicle is composed of a wax and/or a heat-meltible resin as a main ingredient.

Examples of specific waxes include natural waxes such as haze wax, bees wax, lanolin, carnauba wax, candelilla wax, montan wax and ceresine wax; petroleum waxes such as paraffin wax and microcrystalline wax; synthetic waxes such as oxidized wax, ester wax, low molecular weight polyeth-

ylene wax and Fischer-Tropsch wax; higher fatty acids such as lauric acid, myristic acid, palmitic acid, stearic acid and behenic acid; higher aliphatic alcohols such as stearyl alcohol and docosanol; esters such as higher fatty acid monoglycerides, sucrose fatty acid esters and sorbitan fatty acid esters; and amides and besamides such as oleic acid amide. These waxes may be used either alone or in combination.

Examples of specific heat-meltible resins include ethylene copolymers such as ethylene-vinyl acetate copolymer, ethylene-vinyl butyrate copolymer, ethylene-(meth)acrylic acid copolymer, ethylene-alkyl (meth)acrylate copolymer wherein examples of the alkyl group are those having 1 to 16 carbon atoms, such as methyl, ethyl, propyl, butyl, hexyl, heptyl, octyl, 2-ethylhexyl, nonyl, dodecyl and hexadecyl, ethylene-acrylonitrile copolymer, ethylene-acrylamide copolymer, ethylene-N-methylolacrylamide copolymer and ethylene-styrene copolymer; poly(meth)acrylic acid esters such as polylauryl methacrylate and polyhexyl acrylate; vinyl chloride polymer and copolymers such as polyvinyl chloride, vinyl chloride-vinyl acetate copolymer and vinyl chloride-vinyl alcohol copolymer; polyesters, polyamides, cellulose resins, natural rubber, styrene-butadiene copolymer, isoprene polymer, chloroprene polymer, petroleum resins, rosin resins, terpene resins and cumarone-indene resins. These resins may be used either alone or in combination.

As the coloring agent for the monochromatic thermal transfer recording material, usable are carbon black as well as various organic and inorganic pigments.

The coloring agents for yellow, magenta and cyan for the multi-color or full-color thermal transfer recording material are preferably transparent ones.

Examples of specific transparent coloring agents for yellow include organic pigments such as Naphthol Yellow S, Hansa Yellow 5G, Hansa Yellow 3G, Hansa Yellow G, Hansa Yellow GR, Hansa Yellow A, Hansa Yellow RN, Hansa Yellow R, Benzidine Yellow, Benzidine Yellow G, Benzidine Yellow GR, Permanent Yellow NCG and Quinoline Yellow Lake; and dyes such as Auramine. These coloring agents may be used either alone or in combination.

Examples of specific transparent coloring agents for magenta include organic pigments such as Permanent Red 4R, Brilliant Fast Scarlet, Brilliant Carmine BS, Permanent Carmine FB, Lithol Red, Permanent Red F5R, Brilliant Carmine 6B, Pigment Scarlet 3B, Rhodamine Lake B, Rhodamine Lake Y and Arizalin Lake; and dyes such as Rhodamine. These coloring agents may be used either alone or in combination.

Examples of specific transparent coloring agents for cyan include organic pigments such as Victoria Blue Lake, metal-free Phthalocyanine Blue, Phthalocyanine Blue and Fast Sky Blue; and dyes such as Victoria Blue. These coloring agents may be used either alone or in combination.

The term "transparent pigment" is herein meant by a pigment which gives a transparent ink when dispersed in a transparent vehicle.

If the superimposing of the three colors, yellow, magenta and cyan, can hardly give a clear black color, there may be further provided a coated area of a black ink containing a coloring agent for black such as carbon black, Nigrosine Base or the like. The black ink for this purpose is not adapted for the superimposing with other color ink and, hence, need not be necessarily transparent. Nevertheless, the black ink is preferably transparent for the purpose of giving a desired color such as blue black by the superimposing with other color ink.

The content of the coloring agent in the heat-meltable ink for each color is preferably about 5 to 30% by weight.

The heat-meltable ink may be incorporated, in addition to the above ingredients, with a dispersant, an antistatic agent and other additives, as required.

The melting point of the heat-meltable ink is preferably from about 50° to 100° C., more preferably from about 50° to 90° C., still more preferably from about 50° to 85° C. When the melting point is lower than the above range, the storage property of the recording material is prone to degrade. When the melting point is higher than the above range, the transfer sensitivity is prone to degrade.

The coating amount (the value after drying, hereinafter the same) of the ink is preferably from about 1 to 5 g/m<sup>2</sup>.

The thermal transfer recording material of the present invention is preferably applied to a paper sheet having a low surface smoothness, for example, a Bekk smoothness of 50 seconds or less, or a porous surface receptor. In this case, a heat-meltable ink having a melt viscosity of 20 to 200 cps/90° C. is preferably used. Such a low viscosity ink easily permeates into the depressed portions of the paper sheet or the minute pores and depressed portions of the porous surface receptor and images formed from the ink are easily smoothed in the reheating treatment, which results in ink images having excellent abrasion resistance and surface smoothness. When the melt viscosity of the ink is higher than the above range, the ink is difficult to permeate into the depressed portions of the paper sheet or the minute pores and depressed portions of the porous surface receptor and to be smoothed. When the melt viscosity of the ink is lower than the above range, the ink is prone to excessively permeate into the paper sheet or flow on the surface of the porous surface receptor.

The release agent applied to the uncoated areas of the heat-meltable ink on the foundation may be a liquid release agent or a solid release agent. Examples of the liquid release agent are silicone oil, phosphoric acid alkyl esters and fluorine-containing surface active agent. Examples of the solid release agent are silicone resin, silicone-modified urethane resin, silicone-modified acrylic resin and fluorine-containing resin.

The release agent may be applied in the form of a release composition containing the release agent. The release composition comprises a release agent and a binder such as resins. Usable examples of the resin as the binder include nitrocellulose, urethane resin, polyester resin, natural rubber, styrene-butadiene copolymer, isoprene polymer and chloroprene polymer. These resins may be used either alone or in combination. The content of the release agent in the release composition is preferably from 0.5 to 20% by weight.

The coating amount of the release agent is preferably from 0.001 to 5 g/m<sup>2</sup>, more preferably from 0.001 to 1 g/m<sup>2</sup>. When the release agent is liquid, the coating amount thereof is preferably from 0.001 to 0.05 g/m<sup>2</sup>. The coating amount of the release composition is preferably from 0.001 to 5 g/m<sup>2</sup>, more preferably from 0.001 to 1 g/m<sup>2</sup> in terms of the release agent. The coating amount of the release composition is preferably from 0.2 to 5 g/m<sup>2</sup> on the basis of the amount of the release composition itself. When the coating amount of the release agent or release composition is smaller than the above range, the release effect is not sufficiently exhibited in the reheating treatment. When the coating amount is larger than the above range, the heat conduction is prone to degrade, which results in an unfavorable reheating treatment.

The thermal transfer recording material of the present invention exhibits favorable results when being used in

combination with a receptor having a porous surface layer having a large number of minute pores.

Usable as such a porous surface receptor is one disclosed in Japanese Unexamined Patent Publication No. 41287/1990. The porous surface receptor is prepared as follows: Two or more kinds of resins which are immiscible or less miscible with each other (for example, a combination of a homopolymer or copolymer of vinyl chloride and a homopolymer or copolymer of acrylonitrile) is dissolved into a solvent. The solution is applied onto a film substrate such as polypropylene film or polyester film. The resultant is passed through a liquid which is miscible with the solvent and incapable of dissolving the resins, thereby coagulating the resins, followed by drying. Thus a porous resinous layer is formed on the film substrate. The porous resinous layer is brought into contact with a smooth sheet material which is incompatible with the porous resinous layer and subjected to a heating treatment under a pressure to give a receptor having a porous surface layer.

The porous surface layer preferably has an average pore diameter of 0.1 to 10 µm, especially 0.5 to 5 µm, an average pore depth of 0.5 to 15 µm, especially 2 to 10 µm, and an average pore density of 5×10<sup>5</sup> to 1×10<sup>7</sup>/mm<sup>2</sup>.

The porous surface layer preferably has a softening or melting temperature of 40° to 150° C. Such a porous surface layer is softened to be smoothed together with the ink images during the reheating treatment, thereby facilitating smoothing of the ink images. When the softening or melting temperature of the porous surface layer is higher than 150° C., the porous surface layer is not softened in the reheating treatment, resulting in no contribution to the smoothing of the ink images. When the softening or melting temperature of the porous surface layer is lower than the above range, the porous surface layer has tackiness, which causes problems in storage and feeding in a printer.

The present invention will be more fully described by way of Examples. It is to be understood that the present invention is not limited to the Examples, and various changes and modifications may be made in the invention without departing from the spirit and scope thereof.

#### EXAMPLE 1

Onto one side of a 3.5 µm-thick polyethylene terephthalate film which was provided on the other side thereof with a 0.1 µm-thick stick-preventing layer composed of a silicone-modified urethane resin were applied the inks for respective colors each having the composition shown in Table 1 by hot-melt coating. Onto the areas not coated with ink on the film foundation was applied a silicone oil in a coating amount of 0.005 g/m<sup>2</sup>. Thus there was obtained a thermal transfer recording material wherein the coated areas of the different color inks and the coated area of the release agent were arranged as shown in FIG. 2.

TABLE 1

|                                     | Yellow<br>ink | Magenta<br>ink | Cyan<br>ink |
|-------------------------------------|---------------|----------------|-------------|
| Formula (parts by weight)           |               |                |             |
| Paraffin wax                        | 60            | 60             | 60          |
| Carnauba wax                        | 20            | 20             | 20          |
| Ethylene-vinyl<br>acetate copolymer | 5             | 5              | 5           |
| Pigment Yellow                      | 15            | —              | —           |
| Carmine 6B                          | —             | 15             | —           |

TABLE 1-continued

|                                    | Yellow<br>ink | Magenta<br>ink | Cyan<br>ink |
|------------------------------------|---------------|----------------|-------------|
| Cyanine Blue KRO                   | —             | —              | 15          |
| Coating amount (g/m <sup>2</sup> ) | 1.5           | 1.5            | 1.5         |
| Melting point (°C.)                | 71            | 71             | 71          |
| Melt viscosity (cps/90° C.)        | 140           | 140            | 140         |

10

average pore depth: 10 µm, average pore density: 10<sup>6</sup>/mm<sup>2</sup>

The optical reflection density (OD value) was determined 5 with the ink images before and after the reheating treatment. The results are shown in Table 2.

TABLE 2

| Transferred<br>parts | Example 1           |                    | Example 2           |                    | Comparative Example |                    |
|----------------------|---------------------|--------------------|---------------------|--------------------|---------------------|--------------------|
|                      | Before<br>reheating | After<br>reheating | Before<br>reheating | After<br>reheating | Before<br>reheating | After<br>reheating |
| <u>OD value</u>      |                     |                    |                     |                    |                     |                    |
| Y                    | 1.22                | 2.03               | 1.22                | 2.01               | 1.22                | 1.20               |
| M                    | 1.18                | 1.98               | 1.18                | 1.96               | 1.18                | 1.15               |
| C                    | 1.21                | 2.10               | 1.21                | 2.05               | 1.21                | 1.18               |
| Y/M/C                | 1.30                | 1.90               | 1.30                | 1.89               | 1.30                | 1.26               |

25

## EXAMPLE 2

The same procedures as in Example 1 except that a solution of a silicone-modified acrylic resin in methyl ethyl ketone (solid content: 8% by weight) was applied onto the uncoated areas of the inks on the film foundation at a coating amount after drying of 0.2 g/m<sup>2</sup> and dried to give release agent-coated areas were repeated to give a thermal transfer recording material.

Further the transferred parts Y/M, M/C and Y/C after the reheating were evaluated for color reproducibility. All transferred parts provided good color reproducibility.

As described above, when ink images are formed on a porous surface receptor and the ink images are subjected to the reheating treatment by use of the thermal transfer recording material of the present invention, ink images having smooth surface and high density are obtained without reverse transfer. An excellent color reproducibility is exhibited in formation of color ink images.

When ink images are formed on a paper sheet having an uneven surface and the ink images are subjected to the reheating treatment by use of the recording material of the present invention, ink images having excellent abrasion resistance are obtained.

In addition to the materials and ingredients used in the Examples, other materials and ingredients can be used in the Examples as set forth in the specification to obtain substantially the same results.

What is claimed is:

1. A method for forming an image comprising the steps of: providing a thermal transfer recording material comprising a foundation, and (A) a coated area of at least one heat-meltable ink and (B) a coated area of a release agent or a release composition containing a release agent provided on the foundation, the coated area (A) and the coated area (B) being repeatedly arranged in a side-by-side relationship one side of the foundation, the release agent being at least one member selected from the group consisting of a silicone oil, an alkyl phosphate, a fluorine-containing surface active agent, a silicone resin, a silicone-modified urethane resin, a silicone-modified acrylic resin and a fluorine-containing resin,

superimposing the coated area (A) of the recording material onto a receptor having a resinous porous surface layer, and heating the recording material from the back side thereof with a thermal head to selectively melt-transfer the heat-meltable ink of the coated area (A) onto the resinous porous surface layer of the receptor, thereby giving an ink image on the receptor, and superimposing the coated area (B) of the recording material onto the resinous porous surface layer on which the

30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595

ink image has been formed, and heating the recording material from the back side thereof with the thermal head to heat the ink image.

2. The method of claim 1, wherein the resinous porous surface layer of the receptor has an average pore diameter of 0.1 to 10  $\mu\text{m}$ , an average pore depth of 0.5 to 15  $\mu\text{m}$  and an average pore density of  $5 \times 10^5$  to  $1 \times 10^7/\text{mm}^2$ .

3. The method of claim 1, wherein the coated area (A) comprises a coated area of a yellow heat-meltable ink, a coated area of a magenta heat-meltable ink and a coated area of a cyan heat-meltable ink, and at least two of said inks are superimposingly transferred onto the resinous porous surface layer of the receptor in a predetermined order, thereby giving a color image on the basis of subtractive color mixture.

4. The method of claims 3, wherein the coated area (A) further comprises a coated area of a black heat-meltable ink.

5. The method of claim 1, wherein the heat-meltable ink has a melt viscosity of 20 to 200 cps/90° C.

6. The method of claim 1, wherein the coating amount of the release agent in the coated area (B) is from 0.001 to 5 g/m<sup>2</sup>.

10 7. The method of claim 1, wherein the coating amount of the release composition in the coated area (B) is from 0.001 to 5 g/m<sup>2</sup> in terms of the release agent.

\* \* \* \* \*